

# UNITED STATES PATENT OFFICE.

GEORGE W PRIEST, OF WILMINGTON, DELAWARE, ASSIGNOR TO E. I. DU PONT DE NEMOURS & COMPANY, OF WILMINGTON, DELAWARE, A CORPORATION OF DELAWARE.

## LINOLEUM COMPOSITION AND PROCESS OF MAKING SAME.

1,381,738.

Specification of Letters Patent. Patented June 14, 1921.

No Drawing. Original application filed August 8, 1917, Serial No. 185,015. Divided and this application filed September 25, 1918. Serial No. 255,613.

To all whom it may concern:

Be it known that I, GEORGE W. PRIEST, of Wilmington, in the county of New Castle, and in the State of Delaware, have invented 5 a certain new and useful Improvement in Linoleum Compositions and Processes of Making the Same, and do hereby declare that the following is a full, clear, and exact description thereof.

10 My invention relates to plastic compositions containing polymerized coumarone, and to a process of making the same.

The object of my invention is to provide a process of advantageous character for 15 making linoleum compositions, particularly linoleum cements, and the product thereof.

Further objects of my invention will appear from the detailed description thereof contained hereinafter.

20 I have found that when previously polymerized Chinese wood oil or tung oil is ground together in any suitable machine, as for example a machine containing friction rolls, with a polymerized product of the 25 coumarone or indene group of compounds at a temperature of 100° C. or below a material is obtained which has characteristics as to its consistency, combining qualities, solubility, etc., which make it more useful as a 30 cement than in the case where the polymerized product of the coumarone or indene group of compounds is added to the Chinese wood oil when heated to above 100° C.

While my invention is capable of being 35 carried out in many different ways, I shall describe only one example thereof hereinafter.

In order to carry out my process I may for 40 example heat two parts of Chinese wood oil or tung oil to 265° C. so as to polymerize the same and produce a jelly-like material. The material thus obtained is allowed to cool and I then mix therewith one part of a polymerized product of the coumarone or indene 45 group of compounds and grind the same together at a temperature of 100° C. or below thus producing a composition which is elastic, adhesive, coherent and light in color.

This composition may be used for linoleum

cement by mixing with suitable proportions 50 of pigment and ground cork, or woodmeal, as for example

|                                |    |       |
|--------------------------------|----|-------|
| Tung oil coumarone composition | 50 | parts |
| Pigment                        | 20 | "     |
| Ground cork or woodmeal        | 50 | "     |

55 and applying to a fabric by means of pressure. The material may also be used for cementing materials of other kinds together and on fabrics of all kinds.

60 While I have described my invention above in detail, I wish it to be understood that many changes may be made therein without departing from the spirit of the same.

This application is a division of my application Serial No. 185,015, filed August 8, 1917.

I claim:

1. The process which comprises mixing together an oil and a polymerized product 70 of the coumarone or indene group of compounds at a temperature not above 100° C.

2. The process which comprises mixing together an oil and a polymerized product of the coumarone or indene group of compounds 75 and grinding them together between rolls.

3. The process which comprises mixing together an oil and a polymerized product of the coumarone or indene group of compounds 80 at a temperature not above 100° C. and grinding them together between rolls.

4. The process which comprises mixing together polymerized Chinese wood oil and a polymerized product of the coumarone or 85 indene group of compounds at a temperature not above 100° C.

5. The process which comprises mixing together polymerized Chinese wood oil and a polymerized product of the coumarone or 90 indene group of compounds and grinding them together between rolls.

6. The process which comprises mixing together polymerized Chinese wood oil and a polymerized product of the coumarone or 95 indene group of compounds at a temperature not above 100° C. and grinding them together between rolls.

7. A composition of matter comprising an oil mixed and ground together with a polymerized product of the coumarone or indene group of compounds.
- 5 8. A composition of matter comprising polymerized Chinese wood oil mixed and ground together with a polymerized product of the coumarone or indene group of compounds.
- 10 9. The process which comprises mixing together a thickened oil and a polymerized product of the coumarone or indene group of

compounds at a temperature not above 100° C.

10. A composition of matter comprising a 15 thickened oil mixed and ground together with a polymerized product of the coumarone or indene group of compounds.

In testimony that I claim the foregoing I have hereunto set my hand.

GEORGE W. PRIEST.

Witnesses:

G. D. HOPKINS,  
STANLEY L. ABRAMS.